

May 27, 1958

G. A. SAMUEL

2,836,513

CHROMIZING, ADHERING COATING

Filed April 10, 1956



INVENTOR  
George A. Samuel  
BY  
*W. S. Jackson*  
ATTORNEY S.

# United States Patent Office

2,836,513

Patented May 27, 1958

1

2,836,513

## CHROMIZING, ADHERING COATING

George A. Samuel, White Plains, N. Y., assignor to Metal Diffusions, Inc., Philadelphia, Pa., a corporation of New Jersey

Application April 10, 1956, Serial No. 577,297

1 Claim. (Cl. 117—183)

The present invention relates to chromizing of ferrous metal articles, especially sheet, plate and strip steel.

The purpose of the invention is to simplify the chromizing of ferrous metal articles by avoiding the necessity of packing a chromizing compound in a box around the articles.

A further purpose is to permit chromizing ferrous metal articles in existing furnaces or in modified furnaces having atmosphere control.

A further purpose is to accelerate the chromizing of ferrous metal articles by obtaining intimate adherence between a coating of chromizing compound and the surface to be chromized, while at the same time permitting ready removal of the residue which is rendered friable after chromizing.

A further purpose is to employ a stagnant or substantially quiescent relatively light protecting gas which will exert a minimum of washing action which might dissipate heavier chromizing gas.

A further purpose is to place the work in a container or containers open at the top which will trap chromizing gas and prevent its dissipation in the effluent protecting gas.

Further purposes appear in the specification and in the claim.

In the drawings I have chosen to illustrate a few only of the numerous embodiments in which my invention may appear, selecting the forms shown from the standpoints of convenience in illustration, satisfactory operation and clear demonstration of the principles involved.

Figure 1 is a diagrammatic central vertical section of one form of furnace useful in the invention.

Figure 2 is a similar view showing a modification.

Describing in illustration but not in limitation and referring to the drawings:

Chromizing as usually carried out at the present time involves packing of a powdery chromizing composition around ferrous metal articles placed in a chromizing box. Chromizing by this technique is tedious and expensive because of the labor involved in packing, and because of the danger that in certain types of work a high rejection rate may result through inability to obtain uniform and pore free chromizing.

It is particularly difficult to chromize sheet and strip by packing because of the labor involved in spreading the powder in a position to adjoin the side of the sheet.

I have discovered that a relatively simple procedure can be used to obtain uniform, inexpensive chromizing of many ferrous metal articles including sheet, plate and strip. The invention does not require box techniques as at present practiced and lends itself to application in atmosphere heating furnaces, car-bottom furnaces, bell furnaces, muffle furnaces and the like, and on chain and roller hearth furnaces having atmosphere control.

Thus the cost of additional equipment can be reduced to a minimum, while the results obtained are comparable to the best pack methods.

2

The invention is applicable to a wide variety of plain carbon and alloy steels, whether in low, intermediate or high carbon ranges, although for most ductile coatings low carbon is preferred, of the order of 1010. The invention is also applicable to sheet, strip, plate, fabricated forms, wire, rod, bar and tubing, as well as a wide variety of other forms of steel.

In accordance with the invention, an adhering chromizing coating is applied which forms a deposit on the surface of the steel to be chromized. It will be evident, of course, that the coating can be applied by any suitable technique such as roller coating, doctoring, spraying, dipping, brushing, or the like. Where desired, the coating can be applied selectively and if other surfaces are not brought in contact with coating they will not be chromized. For example, one side only of a sheet can be coated and in making a stack the two coated sides of adjoining sheets will be placed together, placing two non-coated sides of adjoining sheets together. The sheets will be chromized then only on one side.

Considering first the form of Figure 1, I make up an adhesive coating or slurry of chromizing compound which has the inherent property of becoming friable by the end of the chromizing operation. The slurry is non-carbonaceous, and therefore has the advantage that it does not carburize the work.

Since the coating is applied directly to the surface of the work, the chromizing gas, which will include fluorine, does not have a tendency to travel great distances in high concentrations, where pickling and etching effects might be obtained, and undergoes a minimum of reactions, but performs very effective transfer of chromium to the work, thus giving better penetration in a given time.

The result is that a minimum of undesired ferrous halide is produced.

The catalyst used is a compound of chromium and fluorine. While any one of the fluorides of chromium may be employed, it is decidedly preferable for several reasons to use a complex chromium ammonium fluoride. One advantage is that this compound breaks down, liberating hydrogen and nitrogen and tending to sweep out air which might otherwise be entrapped adjacent the work. Another advantage is that when the compound breaks down, chromium or chromium and halide is available in nascent form.

While chromium fluoride or a complex ammonium chromium fluoride can be used from any suitable source of such materials, it is preferable to produce the catalyst by a reaction in making the compound. This is desirably accomplished by reacting ammonium bifluoride in water solution with a source of chromium, which may for example be either metallic chromium or ferro chrome in finely divided form. This reaction should be carried out only by an experienced chemist, taking due precautions to deal with explosive conditions, as it occurs violently with evolution of heat and gas, forming the complex ammonium chromium fluoride. There should desirably be an excess of chromium present which will be dispersed in the slurry.

It is also desirable to have an inert powdered bodying ingredient which will prevent close compacting of the chromium particles and prevent sintering at elevated temperatures which might otherwise occur. The inert bodying material may be finely divided alumina, silica or clay, such as kaolin. Any other inert bodying powder may be used.

The slurry or dispersion has some remarkably advantageous properties. When coated by brushing, spraying, dipping or otherwise on the ferrous metal article and allowed to dry, the adhesion is so firm that the work can

undergo even relatively rough handling. This property is very unusual among non-carbonaceous adhesives.

After the chromizing is complete and the complex ammonium fluoride has been broken down, the adhesive action largely disappears and the coating becomes friable and readily flakes off when the work is removed, leaving a clean and clear chromized surface. A convenient way to remove the friable powder is by brushing with a stiff brush.

The preferred embodiment of the invention is a slurry consisting of the following proportions by weight:

|                                                                     | Percent |
|---------------------------------------------------------------------|---------|
| Ammonium bifluoride                                                 | 1.4     |
| Ferro-chromium (preferably the 65 percent by weight chromium grade) | 67.5    |
| Inert bodying ingredient, in this case alumina powder               | 17      |
| Water                                                               | Balance |

In making up this composition, it is preferable to proceed as follows:

Dissolve 10 parts by weight of ammonium bifluoride in 90 parts by weight of water. Make up a mixture of 80 percent by weight of ferro chromium powder and 20 percent by weight of alumina. 6 parts by weight of this mixture is added by stirring to 1 part by weight of the solution of ammonium bifluoride. The violent reaction with evolution of gas and heat continues in some cases for as much as two hours. Allow the resulting slurry to cool. It is then ready for use. If preferred, it can be allowed to dry and then made up with water to its original volume. The dry powder can be shipped as such and mixed with water at a distant point.

There is of course a great excess of chromium in the above mixture and the quantity of ammonium bifluoride is not critical. Good results can be obtained using as little as 0.1 percent by weight of ammonium bifluoride or as much as 10 percent by weight of ammonium bifluoride, adjusting the quantity of water if desired to obtain a suitable slurry.

The slurry should be violently agitated to maintain the ferro chromium powder and the alumina in dispersion when coating the work.

The coating bonds to the work at low temperatures upon drying, and coated articles can be stored for considerable periods before chromizing if desired.

In Figure 1, I illustrate a stack of steel sheets 20 coated with the chromizing compound, in this case on both faces. The stack is placed in a furnace 21 heated in any suitable way, for example by an electric resistance heater 22. The furnace has a door 23 which is kept closed during the operation. An inert protecting gas, preferably hydrogen or split ammonia, but permissibly nitrogen or other suitable inert protecting gas, is used. The inert protecting gas should preferably be a gas whose density is relatively light compared to that of fluorine. The inert protecting gas is preferably introduced at the bottom by pipe 24 and taken out the top by pipe 25.

It is very desirable that the gas stream should be merely great enough to make up for leakage so that a relatively quiescent or stagnant gas atmosphere remains around the work. This protects against removal of fluorine or chromium fluoride vapor by washing or sweeping action which would seriously interfere with the chromizing.

In some cases it is preferable to further protect against dissipation of chromizing gas by placing the work 20 as shown in Figure 2 in a container 26 which is closed at the bottom and sides and open at the top, and suitably has a cover 27 which is not hermetically sealed but merely

loosely fits on the top. This further reduces the possibility of dissipating the chromizing gas by washing or sweeping action since the relatively heavy chromizing gas tends to fill the lower container portion 26.

In Figure 1, the work is shown as a stack of sheets while as in Figure 2 I illustrate the work consisting of a roll of strip held by a band 28. It will be evident that the strip has been suitably coated with chromizing compound while unwound and then after drying has been wound up in roll form.

The chromizing temperature may be between 1600 and 2200 degrees Fahrenheit, preferably between 1650 and 1950 degrees Fahrenheit, and most desirably about 1750 degrees Fahrenheit. The high temperatures are usually to be avoided because of grain growth. The Time of chromizing is suitably in excess of 3 hours, and usually in excess of 5 hours, in many cases being as long as about 18 hours.

The final chromizing coating is bright and firmly adherent, while the powder deposit on the other hand scales off readily.

The improvement in penetration according to the present invention is of the order of 50 to 75 percent over the pack method as normally applied.

The deposit obtained can be of any desired thickness in the range from 0.0001 inch to 0.010 inch. The deposit will commonly be of the order of 0.001 inch.

The particles used in making up the slurry should preferably be through 100 mesh per linear inch.

In operation, it will be evident that it is merely necessary to coat the work with the chromizing compound, allow the compound to dry, then insert the work in the furnace, heat the work up to chromizing temperature, cool the work down to a safe temperature, remove the work from the furnace and then clean off the residual powder. The fact that two articles are touching in a stack or coil is not objectionable, as the powder protects against damage.

In view of my invention and disclosure variations and modifications to meet individual whim or particular need will doubtless become evident to others skilled in the art, to obtain all or part of the benefits of my invention without copying the method shown, and I therefore claim all such insofar as they fall within the reasonable spirit and scope of my invention.

Having thus described my invention, what I claim as new and desire to secure by Letters Patent is:

The method of chromizing ferrous metal articles, which comprises coating the articles with a watery dispersion of chromium, the complex fluoride of ammonium and chromium and an inert bodying agent, to form an adhesive bonded chromizing layer on the ferrous metal articles, and heating the ferrous metal articles to a temperature of 1600 to 2200 degrees F. and maintaining the articles in a closed space at that temperature while exposed to and protected by the gas atmosphere evolved from the complex fluoride to diffuse chromium into the articles and render the coating friable so that it can be easily removed.

#### References Cited in the file of this patent

#### UNITED STATES PATENTS

1,746,924 Bendix Feb. 11, 1930

#### OTHER REFERENCES

"Protective Coatings for Metals," by Burns and Bradley, published by Reinhold (New York), 1955 (page 230 relied on).